

# UNITED STATES PATENT OFFICE.

JESSE R. FITZGERALD, OF TORONTO, ONTARIO, CANADA.

## COMPOSITION FOR FURNITURE AND PIANO POLISHING.

No. 855,451.

Specification of Letters Patent.

Patented June 4, 1907.

Application filed February 28, 1907. Serial No. 359,001.

*To all whom it may concern:*

Be it known that I, JESSE ROLAND FITZGERALD, of the city of Toronto, in the county of York and Province of Ontario, Canada, have invented a certain new and useful Composition for Furniture and Piano Polishing Purposes; and I hereby declare that the following is a full, clear, and exact description of the same.

10 This invention relates to a polish composition for furniture, pianos, and the like, and it consists of forty-one parts of turpentine, ten and one-third parts of black oil, one part of muriatic acid, two-thirds part of butter of 15 antimony, five parts of oil of cedar and forty parts of benzin. The black oil which is one of the non-volatile oils obtained during the distillation of crude petroleum is employed to provide a body and color, and the turpentine is employed as a mixer, for the composition. The black oil and turpentine are first combined and to them is added the muriatic acid and butter of antimony which operate to cut the oily fat in the black oil. 20 To this mixture then is added the benzin and the oil of cedar, the benzin being used to hold the other ingredients suspended to make up the requisite quantity of the polish at the proper consistency, and the oil of cedar being used to produce the requisite gloss. To the above composition may be added two parts of oil of citronella to provide it with a pleasant odor. The ingredients of the composition are then intimately 25 mixed until properly combined.

The composition can be applied in the same manner as other polishes of a like nature

are now applied. When the composition has dried upon the applied surface it can be rubbed in the usual manner until a perfectly 40 smooth and highly polished surface is obtained.

Having thus fully described my invention, what I claim as new and desire to secure by Letters Patent is:

1. A composition for furniture and piano 45 polishing purposes, consisting of a mixture of turpentine, black oil, muriatic acid, butter of antimony, oil of cedar, and benzin.

2. A composition for furniture and piano 50 polishing purposes, consisting of a mixture of turpentine, black oil, muriatic acid, butter of antimony, oil of cedar, benzin and oil of citronella.

3. A composition for furniture and piano 55 polishing purposes, consisting of a mixture of forty-one parts of turpentine, ten and one-third parts of black oil, one part of muriatic acid, two-thirds part of butter of antimony, five parts of oil of cedar and forty parts of 60 benzin.

4. A composition for furniture and piano 65 polishing purposes, consisting of a mixture of forty-one parts of turpentine, ten and one-third parts of black oil, one part of muriatic acid, two-thirds part of butter of antimony, five parts of oil of cedar, forty parts of benzin and two parts of oil of citronella.

Toronto, February 13, 1907.

JESSE R. FITZGERALD.

Signed in the presence of—

CHAS. H. RICHES,  
H. L. TRIMBLE.